

## UNITED STATES PATENT OFFICE.

WILLIAM R. VEAZEY, OF CLEVELAND, OHIO, AND EDWARD C. BURDICK, OF MIDLAND, MICHIGAN, ASSIGNORS TO THE DOW CHEMICAL COMPANY, OF MIDLAND, MICHIGAN, A CORPORATION OF MICHIGAN.

## METHOD OF CASTING LIGHT METAL ALLOYS.

No Drawing. Application filed November 26, 1921, Serial No. 517,948. Renewed April 5, 1923.

To all whom it may concern:

Be it known that we, WILLIAM R. VEAZEY and EDWARD C. BURDICK, both citizens of the United States, and residents of Cleveland, county of Cuyahoga, and State of Ohio, and of Midland, county of Midland, and State of Michigan, respectively, have jointly invented a new and useful Improvement in Methods of Casting Light Metal Alloys, of which the following is a specification, the principle of the invention being herein explained, and the best mode in which we have contemplated applying that principle so as to distinguish it from other inventions.

15 The present improvements relate more particularly to the casting of light metal alloys in which magnesium is the predominant constituent, for example, an alloy such as described in U. S. Patent No. 965,485 to Pistor et al., dated July 26, 1910, containing not less than 80 per cent. of magnesium. By the same token the present improved method or process is, of course, adaptable to the casting of pure magnesium where such metal is handled by itself. The difficulties encountered in handling molten magnesium, or an alloy largely composed of this metal, need not be emphasized, being well recognized, see, for example, U. S. Patent No. 906,820 to Rakowicz, dated December 15, 1908. As best setting forth the state of the art in this connection, attention may further be called to the article by Dr. Ing. Felix Thomas in "Stahl und Eisen", No. 40, page 290 (1920), which affords an authoritative description of the casting of "Elektron" metal as developed by The Chemische Fabrik Griesheim Elektron in Frankfurt.

According to the best known practice, as thus described by Dr. Thomas, such Elektron metal, which is a trade-name applied by the manufacturer in question to a series of light metal alloys containing over 80 per cent. of magnesium with small additions of other metals such as zinc, is melted in wrought iron or cast steel crucibles of limited capacity, such crucibles being closed while being heated in a suitable oven or furnace. Just as soon as all the metal in the crucible has been reduced to molten condition, the crucible is removed from the furnace and its contents poured. However, even where the greatest precautions are taken, it is admitted that a slight overheating of the metal

or other accidents are liable to cause the formation of a black oxide layer, as well as ignition of the mass of molten metal, and the article in question further describes the steps to be taken to extinguish the flame in the crucible if the metal takes fire and to remove the oxide or nitride that results from contact with the atmosphere. Aside from the difficulties just referred to, the method in question involves leaving behind in the crucible a residuum of metal which has to be poured into an iron form and later again melted. The process, in other words, does not lend itself to continuous operation and considerable loss is entailed by thus re-handling the residual portions of the successive batches thus left behind in the crucibles and it is also rendered difficult to maintain the proportion of alloying constituents to accord with any prescribed formula.

One object of the present invention, accordingly, is to provide a method for casting light metal alloys of the class in hand, which will be relatively simple and permit of practically continuous operation for an extended period of time. A further object is to eliminate, to a large degree, the formation of the undesirable oxides and nitrides whereby not only is waste of the valuable magnesium metal avoided, but more perfect castings are secured than has heretofore been possible. To the accomplishment of the foregoing and related ends the invention, then, consists of the steps hereinafter fully described and particularly pointed out in the claims, the following description setting forth but one of the various ways in which the principle of the invention may be carried out.

According to our present improved method or process we employ, instead of a closed crucible in which to melt the magnesium or light metal alloy high in this metal, an open cast iron pot or equivalent suitable vessel in which the metal is melted along with a proper amount of flux, that while heavier than such metal, will have proper surface tension to properly and effectively coat the metal. As an example of such a flux, approximately equal parts of anhydrous magnesium chloride and sodium chloride may be employed, and if the specific gravity of such flux proves inadequate to float the metal after it has been alloyed, a small amount of barium chloride may be

added. After the proper density of the flux has been established and a sufficient body of the molten metal accumulated, the casting is accomplished by directly ladling the metal from the mass floating on the flux, as aforesaid, to the mold. The particular character of the latter, whether a sand mold or permanent mold, e. g., of cast iron, is a matter of indifference so far as the present invention is concerned. In order thus to ladle the metal, the thin film of the flux that overlies the surface of the molten mass of metal in the pot is broken and brushed to one side so as to uncover the clear metal and the ladle can then be filled and lifted before the film is re-established. Where proper precautions are taken, however, such re-establishment of the film will occur before any oxidation or other harmful effect is produced on the exposed metal and by careful manipulation the operator is at the same time able to avoid taking up any of the flux in the ladle. The metal in the latter will, of course, be momentarily exposed to the atmosphere, while it is in the course of transfer from the pot to the mold, but by having the latter in closely juxtaposed relation to such pot, here again we have found that no harmful oxidation occurs, but on the contrary perfect castings can uniformly be obtained with a certainty far exceeding that of any known process.

The temperature of the molten magnesium in the pot, of course, requires to be carefully regulated, but this is a relatively simple operation where the metal is thus floated in an adequate bath of flux of the character described which serves to preserve the metal from direct contact with the walls of the pot to which the heating medium is applied.

The temperature of the molten mass of magnesium may furthermore be regulated by adding fresh stock metal to such floating mass from time to time as the latter is diminished by ladling the metal to the molds. In other words, the mass of the molten metal may be maintained approximately constant and the operation in this way continued indefinitely. The preferred temperature, as just indicated, will be just a trifle above that at which the magnesium, or the particular alloy thereof that is being employed, will melt.

Other modes of applying the principle of our invention may be employed instead of the one explained, change being made as regards the method herein disclosed, provided the step or steps stated by any of the following claims or the equivalent of such stated step or steps be employed.

We therefore particularly point out and distinctly claim as our invention:—

1. In a method of casting magnesium and alloys thereof in which magnesium largely

predominates, the step which consists in melting a quantity of the metal in an open vessel along with a quantity of flux that is heavier than such metal and has a surface tension when in molten state sufficient to cause same to coat the exposed surface of the metal, substantially as described.

2. In a method of casting magnesium and alloys thereof in which magnesium largely predominates, the step which consists in melting a quantity of the metal in an open vessel along with a quantity of flux consisting of a mixture of magnesium chloride and an alkali metal chloride, such flux having a slightly higher specific gravity than such metal and a surface tension when in molten state sufficient to cause same to coat the exposed surface of the metal, substantially as described.

3. In a method of casting magnesium and alloys thereof in which magnesium largely predominates, the step which consists in melting a quantity of the metal in an open vessel along with a quantity of flux consisting of a mixture of magnesium and sodium chlorides in approximately equal proportions, such flux having a slightly higher specific gravity than such metal and a surface tension when in molten state sufficient to cause same to coat the exposed surface of the metal, substantially as described.

4. In a method of casting magnesium and alloys thereof in which magnesium largely predominates, the step which consists in melting a quantity of the metal in an open vessel along with a quantity of flux consisting of a mixture of magnesium and sodium chlorides in approximately equal proportions, with a relatively small amount of barium chloride added, such flux having a slightly higher specific gravity than such metal and a surface tension when in molten state sufficient to cause same to coat the exposed surface of the metal, substantially as described.

5. In a method of casting magnesium and alloys thereof in which magnesium largely predominates, the steps which consist in melting a quantity of the metal, floating same in a bath of flux, and then transferring metal from such floating mass to the mold as required.

6. In a method of casting magnesium and alloys thereof in which magnesium largely predominates, the steps which consist in melting a quantity of the metal, floating same in a bath of flux, and ladling such metal from such floating mass directly to the mold as required.

7. In a method of casting magnesium and alloys thereof in which magnesium largely predominates, the steps which consist in melting a quantity of the metal in a suitable vessel together with a quantity of a flux of slightly higher specific gravity, whereby

such metal is caused to float in a bath of such flux, and ladling such metal from such floating mass directly to the mold as required.

5 8. In a method of casting magnesium and alloys thereof in which magnesium largely predominates, the steps which consist in melting a quantity of the metal in a suitable vessel together with a quantity of a flux 10 of slightly higher specific gravity consisting of a mixture of magnesium chloride and an alkali metal chloride, whereby such metal is caused to float in a bath of such flux, and ladling such metal from such floating 15 mass directly to the mold as required.

9. In a method of casting magnesium and alloys thereof in which magnesium largely predominates, the steps which consist in melting a quantity of the metal in a suitable 20 vessel together with a quantity of a flux of slightly higher specific gravity consisting of a mixture of magnesium and sodium chlorides in approximately equal proportions, whereby such metal is caused to float 25 in a bath of such flux, and ladling such metal from such floating mass directly to the mold as required.

10. In a method of casting magnesium and alloys thereof in which magnesium 30 largely predominates, the steps which con-

sist in melting a quantity of the metal, floating the same in a bath of flux, ladling such metal from such floating mass directly to the mold as required, and adding fresh stock metal to such floating mass as the amount 35 of the latter is thus diminished.

11. A flux for use with molten magnesium and alloys thereof in which magnesium largely predominates, such flux consisting of a mixture of magnesium chloride and an 40 alkali metal chloride in approximately equal proportions with a relatively small amount of barium chloride added to raise the specific gravity of such flux slightly above that of the metal. 45

12. A flux for use with molten magnesium and alloys thereof in which magnesium largely predominates, such flux consisting of a mixture of magnesium and sodium chlorides in approximately equal proportions with a relatively small amount of barium chloride added to raise the specific 50 gravity of such flux slightly above that of the metal.

Signed by me this 21st day of November, 55  
1921.

WILLIAM R. VEAZEY.

Signed by me this 23 day of November,  
1921.

EDWARD C. BURDICK.